

# United States Patent Office

3,198,631

Patented Aug. 3, 1965

1

**3,198,631**  
**MEDIUM DUTY, WEAR RESISTANT MACHINE ELEMENT**

Douglas E. Jones, 1716 7th St. Menominee, Mich.  
No Drawing. Filed May 1, 1961, Ser. No. 106,459  
2 Claims. (Cl. 75—128)

This invention relates to inexpensive, wear resistant elements formed of iron-base, non-magnetic alloys rich in chromium and nickel the structure of which is one of complex carbides in an austenitic matrix, arranged or oriented in the normal dendritic, as cast, form. The elements may be in the forms of valves, valve seat inserts, and other machine elements for use in medium duty applications wherein the elements must retain their hot hardness, resistance to wear, and corrosion resistance, at elevated temperatures. The invention also relates to the compositions from which such machine elements may be formed.

One of the main objects of the invention is the provision of inexpensive medium duty, wear resistant machine elements, such as hard faced or surfaced valves and valve inserts, which may be used in medium duty applications wherein they must be able to withstand medium severe operating temperatures, pressures and corrosive atmospheres without losing their hardness.

Another important object of the invention is the provision of inexpensive alloys for making such medium duty, wear resistant elements which may be used in the as cast condition without heat treatment and have a hardness within the range of about 35 to 45 on the Rockwell "C" scale.

Certain other objects of the invention will be apparent from the following more detailed description and the appended claims.

The machine elements of this invention may be formed of alloys falling within the following general composition:

|            | Percent by weight |
|------------|-------------------|
| Iron       | 45.0-73.0         |
| Chromium   | 12.0-17.0         |
| Nickel     | 12.0-17.0         |
| Silicon    | 1.5-4.0           |
| Molybdenum | 0.0-5.0           |
| Tungsten   | 0.0-5.0           |
| Manganese  | 0.5-2.0           |
| Vanadium   | 0.0-2.5           |
| Carbon     | 1.0-2.5           |

Alloys from which machine elements may be made having excellent properties according to this invention have the following preferred composition:

|            | Percent by weight |
|------------|-------------------|
| Chromium   | 14.50-16.00       |
| Nickel     | 13.50-15.00       |
| Silicon    | 2.00-3.50         |
| Molybdenum | 1 maximum         |
| Tungsten   | 1 maximum         |
| Manganese  | 0.5-0.70          |
| Vanadium   | 0.0-0.5           |
| Carbon     | 1.25-2.00         |
| Iron       | Balance           |

Alloys of the foregoing preferred analysis have been used to make valves and valve inserts for all types of internal combustion engines. These alloys may also be used to make other machine elements which must exhibit good wear resistance under moderately severe operating conditions.

2

The three following formulations falling within the general composition set forth above have the special properties indicated by their respective headings:

|            | MAXIMUM HOT HARDNESS |
|------------|----------------------|
| Chromium   | 15.25-16.00          |
| Nickel     | 13.50-14.25          |
| Silicon    | 2.50-2.75            |
| Molybdenum | 0.75-1.00            |
| Manganese  | 0.60-0.70            |
| Carbon     | 1.90-2.00            |
| Iron       | Balance              |

|            | MAXIMUM HOT STRENGTH |
|------------|----------------------|
| Chromium   | 12.00-12.75          |
| Nickel     | 13.50-14.25          |
| Silicon    | 2.50-2.75            |
| Molybdenum | 1.75-2.25            |
| Tungsten   | 1.75-2.25            |
| Manganese  | 0.75-1.00            |
| Carbon     | 1.90-2.10            |
| Iron       | Balance              |

|            | MAXIMUM DUCTILITY |
|------------|-------------------|
| Chromium   | 14.00-14.75       |
| Nickel     | 14.25-15.00       |
| Silicon    | 2.50-2.75         |
| Tungsten   | 1 maximum         |
| Molybdenum | 1 maximum         |
| Manganese  | 0.50-0.70         |
| Carbon     | 1.10-1.30         |
| Iron       | Balance           |

35 The following specific example will serve to further illustrate how this invention may be practiced.

*Example I*

|    |                                                                         |
|----|-------------------------------------------------------------------------|
| 40 | The following is typical of a production heat of approximately 200 lbs. |
|    | Melt formula: Lbs.                                                      |
| 45 | Nickel metal 28.80                                                      |
|    | ILP pig iron 90.00                                                      |
|    | Mild steel scrap 30.00                                                  |
|    | Low carbon ferrochrome (72% Cr.) 43.60                                  |
|    | Ferrosilicon (83% Si) 3.90                                              |
|    | Ferromanganese (83% Mn.) .50                                            |
| 50 | Ferromolybdenum (62% Mo.) 2.75                                          |
|    | Carbon .32                                                              |

55 (A) Elements and alloys may be melted in any suitable melting device, although induction melting lends itself to better control. Special techniques such as the use of inert atmospheres (i.e. argon) or vacuum may be beneficial but are not generally necessary. Standard deoxidization practices (i.e. ferrosilicon, calcium silicon, etc.) are normally beneficial.

60 (B) This alloy may be cast into almost any type mold material although best results will be obtained with "dry molds" (i.e. shell molds, fired ceramic molds, etc.)

(C) Pouring temperatures will be determined by the complexity of the casting to be produced, its section size or sizes, and mass. Temperatures 250 to 500 degrees F. above the melting point prove most satisfactory. The lower temperature intended for preheated molds or fairly heavy castings and the higher temperature for small castings of thin section in room temperature molds. Melting point of the alloy is approximately 2365 degrees F. more or less depending on composition within the specification.

(D) The above melt formula will produce castings having a composition approximately as follows:

|            |       |
|------------|-------|
| Chromium   | 15.50 |
| Nickel     | 14.40 |
| Silicon    | 2.38  |
| Molybdenum | .82   |
| Manganese  | .58   |
| Carbon     | 1.90  |

(E) Some elements will vary from the composition indicated by an amount dependent on type of melting unit employed, temperatures used, and time consumed in melting, and in some cases the refractory material used for furnace lining.

(F) It should be recognized that the materials used in the melt formula are one combination of many that are possible and permissible (i.e. careful use of secondary metals and analyzed scrap).

What is claimed as new is:

1. A wear resistant valve member for an internal combustion engine formed of an alloy having the following composition:

|            |             |
|------------|-------------|
| Chromium   | 15.25-16.00 |
| Nickel     | 13.50-14.25 |
| Silicon    | 2.50-2.75   |
| Molybdenum | 0.75-1.00   |

|           |           |
|-----------|-----------|
| Manganese | 0.60-0.70 |
| Carbon    | 1.90-2.00 |
| Iron      | Balance   |

2. A wear resistant valve member for an internal combustion engine formed of an alloy having the following composition:

|            |             |
|------------|-------------|
| Chromium   | 12.00-12.75 |
| Nickel     | 13.50-14.25 |
| Silicon    | 2.50-2.75   |
| Molybdenum | 1.75-2.25   |
| Tungsten   | 1.75-2.25   |
| Manganese  | 0.75-1.00   |
| Carbon     | 1.90-2.10   |
| Iron       | Balance     |

References Cited by the Examiner

UNITED STATES PATENTS

1,745,360 2/30 Silva et al. 75-128

FOREIGN PATENTS

545,377 8/57 Canada.

DAVID L. RECK, Primary Examiner.

MARCUS U. LYONS, RAY K. WINDHAM, Examiners.